# EUROPEAN PATENT SPECIFICATION

(11) **EP 1 367 152 B1**
(45) Date of publication and mention of the grant of the patent: **04.01.2006**
(21) Application number: 03009793.5
(22) Date of filing: 09.05.2003
(51) Int. Cl.: D01F 1/10, D04H 1/42, D04H 1/54, D04H 1/56, D04H 3/14, D04H 3/16, D04H 5/06

(54) **Method for producing a non-woven fabric made of synthetic fiber with fragrancing means**
Methode zur Herstellung eines Vliesstoffes aus synthetischen Fasern mit Duftmittel
Méthode pour produire un non-tissé à base de fibres synthétiques parfumées

(30) Priority: 28.05.2002 IT MI20021155
(43) Date of publication of application: 03.12.2003
(73) Proprietor: Atex S.r.l., 20090 Settala (Prov. of Milan) (IT)
(72) Inventor: Castellani, Massimiliano, 20129 Milan (IT); Ferranti, Silvia, 26010 Dovera (Lodi) (IT)
(74) Representative: Modiano, Micaela Nadia

(56) References cited:
- US-A- 3 852 401
- US-A- 4 713 291
- PATENT ABSTRACTS OF JAPAN vol. 014, no. 053 (C-0683), 31 January 1990 (1990-01-31) & JP 01 282305 A (KURARAY CO LTD), 14 November 1989 (1989-11-14)
- PATENT ABSTRACTS OF JAPAN vol. 017, no. 420 (C-1093), 5 August 1993 (1993-08-05) & JP 05 086501 A (ASAHI CHEM IND CO LTD), 6 April 1993 (1993-04-06)
- PATENT ABSTRACTS OF JAPAN vol. 014, no. 406 (C-0754), 4 September 1990 (1990-09-04) & JP 02 154007 A (ASAHI CHEM IND CO LTD), 13 June 1990 (1990-06-13)

## Description

The present invention relates to a method for producing a non-woven fabric made of synthetic fiber with fragrancing means.

As is known, in order to give a non-woven fabric made of extruded thermoplastic fiber the characteristic of releasing a fragrance, methods are currently used which apply a finishing that contains the fragranced material, that provide for the fixing thereof on the web of non-woven fabric, or for the coextrusion of the fragrancing product during the formation of the layer.

With the finishing methods currently in use, there is a considerable loss of fragrance due to its incompatibility with plastic material and accordingly there is a reduced persistence of the fragrance on the web due to its high evaporability.

In the case of coextrusion with the plastic substrate, the low amount of fragranced material absorbed during the extrusion step is unable to ensure its persistence over time; moreover, the fragrancing substance can break the filament due to its high vapor pressure or sublimation.

Because of the difficulties noted above, the methods currently used to produce a fragranced web of fiber have yielded highly unsatisfactory results; moreover, the fragrances that can be used for this type of application are limited in their olfactory qualities due to the problems of the support material and to the negative action of the extrusion temperature that it was necessary to use.

JP 01 282305 A discloses obtaining an aromatic fibre having a prescribed aroma by homogeneously dispersing and mixing microcapsule powder containing a perfume with a polyester based compound; adding the resulting mixture to a molten polymer fluid of a thermoplastic polymer; knitting in a static mixer such polymer; discharging it from a spinning nozzle and forming it into a fibre.

The aim of the invention is to solve the problem noted above, by providing a method for producing a non-woven fabric made of synthetic fiber with fragrancing means that allows to provide a non-woven fabric, in the form of a web, which contains a fragranced essence that can release a fragrance for a long period of time.

Within this aim, an object of the invention is to provide a method in which the introduction of the fragrancing substance does not entail a degradation of the mechanical properties of the filament and is also capable of giving excellent mechanical properties, thus allowing to provide webs of non-woven fabric that are suitable for many fields of application, such as for example absorbent diapers and incontinence diapers, curtains, household products and the like.

Another object of the present invention is to provide a method that allows hitherto impossible applications, with a wide range of usable fragrances.

Another object of the present invention is to provide a method that can be obtained easily starting from commonly commercially available elements and materials and is also competitive from a merely economical standpoint.

This aim and these and other objects that will become better apparent hereinafter are achieved by a method for producing a non-woven fabric made of synthetic fiber with fragrancing means, according to the invention, characterized in that it comprises providing a melted mass of thermoplastic resin, in introducing in said mass a base mix that contains microcapsules of fragranced substance, in extruding said mass, in stretching the extruded filaments, and in providing a web of non-woven fabric by means of said extruded filaments.

Further characteristics and advantages will become better apparent from the description of a preferred but not exclusive embodiment of a method for producing a non-woven fabric made of synthetic fiber with fragrancing means, illustrated with the aid of the following description.

The method for producing a non-woven fabric made of synthetic fiber with fragrancing means, according to the invention, comprises providing a melted mass of thermoplastic resin, which is advantageously selected from polypropylene, polyethylene, polyester, or other suitable plastic materials.

As a particular characteristic of the invention, an odorous or fragrancing substance is introduced in the melted mass; such substance is constituted by a base mix that contains microcapsules or microspheres of the selected fragrancing substance, which is constituted, for example, by an Accurel Fragrance, provided by Akzo Nobel.

The base mix is first master-batched in a compound that uses the same thermoplastic resin with which the web is to be produced; experimental tests that have been conducted have shown that the base mix must advantageously contain approximately 10-70% by weight of the melted mass of fragrance microcapsules.

The fragrance is preferably, advantageously selected from materials with a high boiling point, so that it can withstand without any variation or degradation the normal operating temperatures during the extrusion step.

During the extrusion step, the base mix, as described above, is introduced in an amount with a percentage from 0.2 to 5% by weight with respect to the total weight of the melted mass.

The base mix is obtained by using the selected type of fragrance, which is placed in microspheres or microcapsules with a size of less than one micron, and is dispersed in the thermoplastic resin that is used.

During extrusion and the subsequent steps of operation, the processing conditions are selected so that the microspheres remain mostly intact in the filament of the fabric and allow the fragrancing substance to release the fragrance for a long period of time.

It has been found out that containing the fragrance in microcapsules effectively prevents its thermal degradation.

The extrusion temperature of the thermoplastic resins is selected to be between 230 and 270 °C, thus achieving complete amalgamation of the two substances and performing a spinning that is totally free from filament breakage.

In the case of polypropylene, it is convenient to use polypropylene of the Finapro 10099 type provided by Atofina, or equivalents from the companies Basell and Amoco, which have a melt index in the interval between 20 and 40 (g/10 min 230 °C 2.16 kg).

The method comprises extruding the mass of resin with the microcapsules of fragrancing substance introduced therein, the various filaments being extruded in continuous form and stretched, advantageously, by means of a stream of compressed air in order to obtain a filament count between 1 and 4 dtex.

The extruded filaments are further spread and crossed on a rotating mat, obtaining a web of non-woven fabric that is bonded by using two hot rollers, one of which is embossed.

The bonding temperature remains in the interval between 120 and 180 °C.

The resulting web of non-woven fabric is further subsequently collected in rolls ready for subsequent processing.

Preferably, the extruded filaments must have a count of no less than 0.5 dtex, since with lower values frequent breakages of the filament are possible, due to the dimensions of the microcapsules, which would be greater, for example in cross-section, than the filament.

Experimental tests that have been conducted have shown that introducing the microcapsules of fragranced substance, in accordance with the described method, does not have particular effects on the characteristics of the resulting fabric, as regards elongations and breaking tenacity both transversely and longitudinally.

Tests have been conducted experimentally by introducing a base mix in an amount of 0.2, 0.5, 1, 2.5 and 5%; the resulting non-woven fabric, with a grammage of 40 g/m², exhibited characteristics of transverse and longitudinal tenacity and elongation that are fully equivalent to those of the similar non-woven fabric without the additive agent or addition of the master mix.

It appears , therefore, that the tests for tenacity and breaking elongation of the non-woven fabric with the addition of the microcapsules of fragranced substance show no substantial differences with respect to the tests of the material without the additive. It is therefore correct to assume that the addition of the master mix, with the described method, does not change substantially the characteristics of the resulting product.

From what has been illustrated above it is evident that the invention achieves the intended aim and objects, and in particular the fact is stressed that with the method described above it is possible to obtain a web of non-woven fabric that has fragrancing characteristics and is particularly suitable for applications in various fields and particularly in the production of absorbent diapers and incontinence diapers, curtains, and household products and the like.

The invention thus conceived is susceptible of numerous modifications and variations, all of which are within the scope of the appended claims.

All the details may further be replaced with other technically equivalent elements.

In practice, the materials used, so long as they are compatible with the specific use, as well as the contingent shapes and dimensions, may be any according to requirements.

## Claims

1. A method for producing a non-woven fabric made of synthetic filaments with fragrancing means, comprising the steps of providing a melted mass of thermoplastic resin, introducing in said mass a base mix that contains microcapsules of fragranced substance, extruding said mass to obtain extruded filaments in continuous form, stretching the extruded filaments and further spreading and crossing said extruded filaments on a rotating mat to obtain a web of non-woven fabric by bonding, by way of hot rollers, the bonding temperature being selected in an interval between 120 and 180 °C.

2. The method according to claim 1, **characterized in that** said base mix is first master-batched in a compound that uses the same thermoplastic resin to be extruded and said microcapsules of fragrancing substance in a percentage between 10 and 70% by weight.

3. The method according to one or more of the preceding claims, **characterized in that** said fragrancing substance is selected from fragrancing substances with a high boiling point.

4. The method according to one or more of the preceding claims, **characterized in that** said base mix is introduced in a percentage from 0.2 to 5% by weight with respect to the total weight of the melted mass.

5. The method according to one or more of the preceding claims, **characterized in that** said fragrancing substance is placed in microcapsules having a size of less than one micron.

6. The method according to one or more of the preceding claims, **characterized in that** said thermoplastic resins are extruded at a temperature between 230 and 270 °C.

7. The method according to one or more of the preceding claims, **characterized in that** said thermoplastic resin is constituted by polypropylene.

8. The method according to one or more of claims 1-6, **characterized in that** said thermoplastic resin is constituted by polyester.

9. The method according to one or more of claims 1-6, **characterized in that** said thermoplastic resin is constituted by polyethylene.

10. The method according to one or more of the preceding claims, **characterized in that** said extruded filaments have a count of more than 0.5 dtex.

## Patentansprüche

1. Verfahren zur Herstellung eines Vliesstoffs, der aus synthetischen Fasern mit Duftmitteln besteht, umfassend die Schritte des Bereitstellens einer geschmolzenen Masse aus thermoplastischem Harz, des Einführens eines Basisgemisches, das Mikrokapseln eines Duftstoffs enthält, in die Masse, des Extrudierens der Masse, um extrudierte Fasern in kontinuierlicher Form zu erhalten, des Dehnens der extrudierten Fasern und des weiteren Ausbreitens und Kreuzens der extrudierten Fasern auf einer Drehmatte, um durch Binden mittels Heißwalzen eine Bahn aus Vliesstoff zu erhalten, wobei die Bindetemperatur in einem Intervall zwischen 120 und 180°C ausgewählt wird.

2. Verfahren nach Anspruch 1, **dadurch gekennzeichnet, daß** das Basisgemisch zuerst in einer Verbindung vorgemischt wird, die dasselbe zu extrudierende thermoplastische Harz und die Mikrokapseln des Duftstoffs in einem Prozentsatz zwischen 10 und 70 Gewichts-% verwendet.

3. Verfahren nach einem oder mehreren der vorangehenden Ansprüche, **dadurch gekennzeichnet, daß** der Duftstoff aus Duftstoffen mit einem hohen Siedepunkt ausgewählt wird.

4. Verfahren nach einem oder mehreren der vorangehenden Ansprüche, **dadurch gekennzeichnet, daß** das Basisgemisch in einem Prozentsatz von 0,2 bis 5 Gewichts-% in Bezug auf das Gesamtgewicht der geschmolzenen Masse eingeführt wird.

5. Verfahren nach einem oder mehreren der vorangehenden Ansprüche, **dadurch gekennzeichnet, daß** der Duftstoff in Mikrokapseln mit einer Größe von weniger als einem Mikrometer angeordnet ist.

6. Verfahren nach einem oder mehreren der vorangehenden Ansprüche, **dadurch gekennzeichnet, daß** die thermoplastischen Harze bei einer Temperatur zwischen 230 und 270°C extrudiert werden.

7. Verfahren nach einem oder mehreren der vorangehenden Ansprüche, **dadurch gekennzeichnet, daß** das thermoplastische Harz aus Polypropylen besteht.

8. Verfahren nach einem oder mehreren der Ansprüche 1-6, **dadurch gekennzeichnet, daß** das thermoplastische Harz aus Polyester besteht.

9. Verfahren nach einem oder mehreren der Ansprüche 1-6, **dadurch gekennzeichnet, daß** das thermoplastische Harz aus Polyethylen besteht.

10. Verfahren nach einem oder mehreren der vorangehenden Ansprüche, **dadurch gekennzeichnet, daß** die extrudierten Fasern eine Fadenstärke von mehr als 0,5 dtex aufweisen.

## Revendications

1. Procédé pour produire une étoffe non-tissée formée de filaments synthétiques avec des moyens parfumeurs, comprenant les étapes consistant à fournir une masse fondue de résine thermoplastique, introduire dans ladite masse un mélange de base qui contient des microcapsules de substance parfumée, extruder ladite masse pour obtenir des filaments extrudés sous forme continue, étirer les filaments extrudés et ensuite étaler et croiser lesdits filaments extrudés sur un matelas rotatif pour obtenir un voile d'étoffe non-tissée par liaison, par le biais de rouleaux chauds, la température de liaison étant choisie dans un intervalle entre 120 et 180°C.

2. Procédé selon la revendication 1, **caractérisé en ce que** ledit mélange de base est obtenu en formant d'abord un mélange maître d'un composé qui utilise la même résine thermoplastique à extruder et desdites microcapsules de substance parfumeuse dans un pourcentage entre 10 et 70 % en poids.

3. Procédé selon l'une ou plusieurs des revendications précédentes, **caractérisé en ce que** ladite substance parfumeuse est choisie parmi les substances parfumeuses ayant un point d'ébullition élevé.

4. Procédé selon l'une ou plusieurs des revendications précédentes, **caractérisé en ce que** ledit mélange de base est introduit dans un pourcentage de 0,2 à 5 % en poids par rapport au poids total de la masse fondue.

5. Procédé selon l'une ou plusieurs des revendications précédentes, **caractérisé en ce que** ladite substance parfumeuse est placée dans des microcapsules ayant une taille de moins de un micron.

6. Procédé selon l'une ou plusieurs des revendications précédentes, **caractérisé en ce que** lesdites résines thermoplastiques sont extrudées à une température entre 230 et 270°C.

7. Procédé selon l'une ou plusieurs des revendications précédentes, **caractérisé en ce que** ladite résine thermoplastique est constituée par du polypropylène.

8. Procédé selon l'une ou plusieurs des revendications 1 à 6, **caractérisé en ce que** ladite résine thermoplastique est constituée par du polyester.

9. Procédé selon l'une ou plusieurs des revendications 1 à 6, **caractérisé en ce que** ladite résine thermoplastique est constituée par du polyéthylène.

10. Procédé selon l'une ou plusieurs des revendications précédentes, **caractérisé en ce que** lesdits filaments extrudés ont un numéro de finesse de plus de 0,5 dtex.
